

## UNITED STATES PATENT OFFICE

2,187,742

## LUBRICANT

James W. Johnson, Philadelphia, Pa., assignor to  
 The Atlantic Refining Company, Philadelphia,  
 Pa., a corporation of Pennsylvania

No Drawing. Application May 12, 1938,  
 Serial No. 207,508

6 Claims. (Cl. 87—9)

The present invention relates to improvements in lubricating oils and more particularly to a method for increasing their lubricity or "oiliness".

It has generally been known that the quality of a lubricating oil depends on some properties other than the viscosity of the hydrocarbon oil. This has been found to be particularly true when the lubricant is used under conditions of thin film or boundary lubrication in which the layer 10 of lubricating oil between the rubbing surfaces is very thin. It has been found that some oils act as better lubricants than others under conditions of boundary lubrication even though their viscosities at the temperature of use are substantially the same. The property of one oil which makes it a better lubricant than another under these conditions, particularly in lowering friction and/or wear, has been designated as "oiliness".

20 It is therefore an object of this invention to increase the "oiliness" of paraffin base, mixed base and naphthalene base lubricating oils by the addition thereto of a relatively small proportion of a material which is active to improve this property 25 without objectionably affecting other desirable properties thereof. More particularly, the present invention relates to the production of an improved lubricating oil of this type having increased "oiliness" by the addition thereto of a urethane. By the term "urethane" is meant the esters of carbamic acid and substituted derivatives thereof.

In accordance with my invention, a urethane or a mixture of urethanes is admixed with a lubricating oil in quantities of the order of 0.1%, 35 0.25%, 0.5% or 1% by weight, or more, depending upon the degree of improvement desired. Among the urethanes which may be suitably employed are methyl urethane, ethyl urethane, ethylene urethane, propyl urethane, butyl urethane, amyl urethane, allyl urethane, acetyl urethane, nitrosourethane, nitrosomethyl urethane, nitro urethane, methyl nitro urethane and the like.

40 In order to determine the effectiveness of the urethanes as addition agents for improving the "oiliness" of lubricating oil, small quantities were added to a hydrocarbon oil having a Saybolt Universal viscosity of 376 seconds at 100° F., an A. P. I. gravity of 21.9, and containing 3% by volume of tricresyl phosphate. The latter material has little or no effect upon the "oiliness" but functions to increase the film strength of the oil and permit "oiliness" tests to be carried on under heavier loads than the hydrocarbon lubricating oil, per se, is able to withstand. The determina-

tion of the "oiliness" or lowering of the coefficient of friction was made in an Almen extreme pressure lubricant testing machine at 200 R. P. M., the load being expressed in lbs./sq. in. projected bearing area and the "oiliness" as a measure of the friction expressed in pound-feet torque.

| Lubricant                                                            | Load (lbs./sq. in.) |         |         |         | 10 |
|----------------------------------------------------------------------|---------------------|---------|---------|---------|----|
|                                                                      | 10,000              | 15,000  | 20,000  | 22,000  |    |
|                                                                      | Lb.-Ft.             | Lb.-Ft. | Lb.-Ft. | Lb.-Ft. |    |
| Oil + 3% tricresyl phosphate                                         | 35                  | 48      | 58      | 60      |    |
| Oil + 3% tricresyl phosphate + 1% urethane                           | 28                  | 38      | 49      | 53      |    |
| Oil + 3% tricresyl phosphate + 0.25% butyl urethane                  | 30                  | 39      | 47      | 49      | 15 |
| Oil + 3% tricresyl phosphate + 0.5% butyl ethyl imido di-carboxylate | 30                  | 41      | 48      | 50      |    |

From the above table it will be seen that the addition of a urethane or substituted urethane to a lubricating oil improves the "oiliness" or reduces friction to a substantial extent. It is not necessary that the lubricant contain a film strength addition agent such as tricresyl phosphate, since an unblended hydrocarbon lubricating oil will exhibit a marked improvement in "oiliness" simply upon the addition of a urethane or substituted urethane such as hereinbefore mentioned. In the event that increased film strength is likewise desired, there may be added to the oil-urethane blend, a quantity of film strength agent such as aliphatic or aromatic phosphates, phosphites or thiophosphates, chlorinated esters or chlorinated hydrocarbons, or other known agents for improving film strength.

For brevity, in the appended claims, the term "a urethane" is to be understood to comprehend urethane and substituted urethanes, or mixture of two or more of them.

What I claim is:

1. A lubricant comprising a hydrocarbon oil and a small amount of a urethane.
2. A lubricant comprising a hydrocarbon oil and less than substantially 1% by weight of a urethane.
3. A lubricant comprising a hydrocarbon oil and a small amount of an alkyl urethane.
4. A lubricant comprising a hydrocarbon oil and a small amount of ethyl urethane.
5. A lubricant comprising a hydrocarbon oil and a small amount of butyl urethane.
6. A lubricant comprising a hydrocarbon oil and a small amount of butyl ethyl imido dicarboxylate.

JAMES W. JOHNSON. 55